

April 9, 1935.

L. D. MANNES ET AL

1,996,928

SENSITIZED PHOTOGRAPHIC ELEMENT AND PROCESS OF MAKING SAME

Filed March 19, 1930

PREPARATION

Fig. 1,



Emulsion in Gelatin — Silver halide precipitated in presence of color forming compound.

BEFORE EXPOSURE

Fig. 2,



Gelatin containing particles of silver halide with absorbed or adsorbed color-forming compound.

AFTER EXPOSURE

Fig. 3,



Gelatin containing silver halide emulsion with adsorbed or adsorbed color forming material — some parts of which have been exposed to light

AFTER DEVELOPMENT

Fig. 4,



Particles of silver with adsorbed or adsorbed color forming material suspended in gelatin

AFTER REMOVAL OF SILVER

Fig. 5.



Particles of colored material suspended in the gelatin  
Silver dissolved out

LEGEND:

Sensitive silver halide with adsorbed or adsorbed color former.

Ditto after exposure to light.

Ditto reduced to silver by development.

Color material after silver has been dissolved out.

INVENTORS:

L. D. Mannes & J. Podowsky, Jr.

BY:

Bruce Davis Mason & Daniels,

THEIR ATTORNEYS.

## UNITED STATES PATENT OFFICE

1,996,928

SENSITIZED PHOTOGRAPHIC ELEMENT AND  
PROCESS OF MAKING SAMELeopold D. Mannes and Leopold Godowsky, Jr.,  
New York, N. Y.

Application March 19, 1930, Serial No. 437,266

14 Claims. (Cl. 95—2)

The invention of this application relates to light-sensitive photographic elements and to methods of making and of using the same.

The principal object of the invention is to provide a photographic element by means of which a photographic image in color may be obtained by a direct and single development.

The invention may be employed for the production of pictures in natural color by using two colors corresponding to the two colors of a "two-color" process or by using three colors corresponding to the three colors of a "three-color" process. Also four or more different colors may be employed but ordinarily three colors are the maximum number required.

The invention is illustrated in the accompanying drawing in which:

Fig. 1 shows diagrammatically the silver halide emulsion.

Fig. 2 shows the colored emulsion prior to exposure.

Fig. 3 shows the exposed plate or film.

Fig. 4 shows the developed plate or film; and

Fig. 5 shows the completed product with the silver removed.

The invention may also be employed for the production of pictures in a single color, that is to say, instead of coloring the silver image by toning or dyeing, there may be produced by the invention a colored picture wherein the image is formed of an insoluble colored compound suspended in the colloidal compound forming the body of the emulsion. The invention is based on the fact that light-sensitive silver halides may be formed by precipitating them in the presence of certain organic compounds such as alpha naphthol or paranitrobenzylcyanide, these latter compounds being absorbed by or adsorbed to the silver-halide crystal or grains thus formed. When these grains, distributed in an ordinary emulsion, that is, suspended in a colloidal medium, are exposed in the course of the customary photographic process and developed by such a developer as diethyl paraphenylenediamine hydrochloride, there is formed in situ with the reduced silver image and by the local oxidation reaction of the development a substantially insoluble colored compound which will remain suspended in whatever colloidal medium holds the halide grain. The silver image itself furthers the reaction apparently by catalysis.

This process is to be distinguished from previously described processes in which the color-forming compound is merely dispersed, among the silver halide grains suspended in the colloid; the

silver halide grains in this case here disclosed adsorbing or absorbing the color-forming compound in question instead of allowing it to permeate the colloid indiscriminately. This process is to be further distinguished from others previously attempted in which highly colored compounds were precipitated in combination with the silver halide. An emulsion thus formed would be sufficiently absorptive to light of certain colors, to prohibit normal penetration of incident light necessary to correct exposure. These color-forming compounds here referred to are all substantially colorless, especially in the minute quantities employed for this purpose, thus not materially affecting the normal color of an emulsion.

After development, the silver may be removed with potassium-cyanide, for instance, leaving a pure colored image. Potassium ferricyanide and hypo may be used instead of potassium cyanide.

If a single emulsion is employed containing grains of silver halide with a single absorbed or adsorbed color-former, there will be produced by the procedure described a picture in the color desired, depending on the particular color-former employed in the manufacture of the film. Thus with the same developer and the same procedure of development a variety of different color effects may be obtained. The selection of the desired color is made by selecting the particular film to be exposed. The color of the resulting picture will be designated on the film package and the user has merely to select the film for the desired color and follow the ordinary procedure of development as above described.

The invention may be employed in color photography in several different ways.

We preferably intermix a plurality of differently color-sensitized emulsions containing respectively different color-formers and apply the mixture in a single layer to the support. A single exposure followed by a single development of such a film will cause each color record to be developed to a correspondingly different color.

For a two-color process a red-sensitive emulsion containing a silver halide precipitated with trichloronaphthol or related compound and a blue-green sensitive emulsion containing a silver halide precipitated with a nitrobenzylcyanide compound mixed with, say, ethyl acetoacetate, are intermixed and spread on the film or other support in a single layer. The film is exposed in the usual manner and developed with a developer such as diethyl paraphenylenediamine hydrochloride. Both images are thus simultaneously developed, and also there are simultane-

ously formed two color images corresponding to the silver images. The silver images are thereafter dissolved out leaving clear colored images.

A third layer may be coated for tri-color recording consisting of an ordinary blue-sensitized (i. e. not especially sensitized) layer containing yellow filter dye, the grains of this layer containing a yellow color-former such as ethyl-acetoacetate. This compound will in such an instance be left out of the green-sensitive layer. In the case of emulsion mixtures such a third emulsion may be mixed together with the two described above.

Instead of mixing the emulsions they may be applied in separate layers, preferably with the red-sensitive layer next the film. No change need be made in the exposure, development and subsequent treatment of the film. The two images will be simultaneously formed as before.

Similar positives may be produced by printing from the negatives on positive film of the same character, with the emulsions either admixed or in separate layers, and thereafter following the same procedure of development, etc.

The term "color-former" here used refers to organic compounds acting as couplers in connection with certain developers in photographic processes, thus forming colored compounds, usually insoluble in water, in the presence of the finely divided silver being reduced by the developing agent. This, in general, distinguishes them from leuco-bases and rather classifies them as intermediate couplers in a dye-forming process. Phenols, naphthols, cresols, nitrophenylacetetonitriles, ethyl acetoacetate, and their halogenated or sulphonic acid compounds are typical members of this type of color-former.

Paraphenylenediamines and paramidophenols are typical developers used in conjunction with the color-formers.

The colored compounds so formed belong to the class, for instance, of indophenols, indoanilines, and indamines.

We claim:

1. A light-sensitive photographic emulsion comprising a colloidal carrier containing silver halide grains, certain of said grains carrying an absorbed or adsorbed color-forming compound.

2. A light-sensitive photographic emulsion comprising a colloidal carrier containing silver halide grains, certain of said grains carrying an absorbed or adsorbed substantially colorless substance adapted when subjected to the action of a developer to produce a substantially insoluble colored compound suspended in a colloidal carrier.

3. A light-sensitive photographic emulsion comprising a colloidal carrier containing silver halide grains, certain of said grains carrying an

absorbed or adsorbed substance adapted when subjected to the action of a developer to produce a substantially transparent insoluble compound of a color not theretofore present in said substance suspended in a colloidal carrier.

4. The method of making a light-sensitive photographic element which consists in precipitating a silver halide in the presence of an organic color-forming compound, and thereafter distributing said precipitate in a suitable emulsion 10 or other colloidal medium.

5. A light-sensitive photographic element which consists of a support, an emulsion thereon, said emulsion containing a plurality of different light-sensitive substances, each substance 15 comprising a silver halide with an absorbed or adsorbed color-former, the color-formers of the different light-sensitive substances being adapted to produce different colors.

6. A silver halide grain or crystal with an absorbed or adsorbed color-forming compound.

7. The method of producing a silver halide grain or crystal with an absorbed or adsorbed color-former, which consists in precipitating the silver halide in the presence of a color-former.

8. The method of producing a silver halide grain or crystal with an absorbed or adsorbed color-former, which consists in ripening the silver halide in the presence of a color-former.

9. A silver halide grain or crystal with an absorbed or adsorbed color-forming compound, said halide being also sensitized to record a particular color or set of colors.

10. The method of producing a silver halide grain or crystal with an absorbed or adsorbed 35 color-former, which consists in precipitating the silver halide in the presence of a color-former and subjecting it to the action of a color-sensitizer.

11. A light-sensitive grain or crystal containing silver, with a color-forming compound bound thereto by physical or chemical union.

12. The method of producing the grain or crystal of the foregoing claim which consists in precipitating the light-sensitive silver compound 45 in the presence of a color-former.

13. A light-sensitive grain or crystal containing silver, with a color-forming compound bound thereto by physical or chemical union, said grain or crystal being sensitized to record a particular 50 color or set of colors.

14. The method of producing the grain or crystal of the preceding claim which consists in the precipitating of the silver compound in the presence of a color-former and subjecting it to 55 the action of a color-sensitizer.

LEOPOLD D. MANNES.

LEOPOLD GODOWSKY, JR.